# EUROPEAN PATENT SPECIFICATION

(11) **EP 3 001 519 B1**
(45) Date of publication and mention of the grant of the patent: **01.05.2019**
(21) Application number: 14801406.1
(22) Date of filing: 21.05.2014
(51) Int. Cl.: H01T 21/02

(54) **METHOD FOR MANUFACTURING SPARK PLUG FOR INTERNAL COMBUSTION ENGINE**
VERFAHREN ZUR HERSTELLUNG EINER ZÜNDKERZE FÜR EINEN VERBRENNUNGSMOTOR
PROCÉDÉ DE PRODUCTION DE BOUGIE D'ALLUMAGE POUR MOTEUR À COMBUSTION INTERNE

(30) Priority: 21.05.2013 JP 2013106942
(43) Date of publication of application: 30.03.2016
(73) Proprietor: DENSO CORPORATION, Kariya-city, Aichi-pref. 448-8661 (JP); Tanaka Kikinzoku Kogyo K.K., Chiyoda-ku Tokyo 100-6422 (JP)
(72) Inventor: MURAYAMA, Yuki, Kariya-city Aichi 448-8661 (JP); ABE, Nobuo, Kariya-city Aichi 448-8661 (JP); SAKAIRI, Koichi, Hiratsuka-shi Kanagawa 254-0076 (JP); TANAKA, Kunihiro, Hiratsuka-shi Kanagawa 254-0076 (JP)
(74) Representative: Kuhnen & Wacker Patent- und Rechtsanwaltsbüro PartG mbB
(86) International application number: PCT/JP2014/063507
(87) International publication number: WO 2014/189088

(56) References cited:
- JP-A- 2008 077 838
- JP-A- 2009 533 803
- US-A1- 2007 114 900
- US-A1- 2008 074 025

## Description

### [TECHNICAL FIELD]

The present invention relates to a method of manufacturing a spark plug for an internal combustion engine; in the spark plug, at least one of a center electrode and a ground electrode includes a discharge chip, the center and ground electrodes being opposed to each other with a spark discharge gap formed therebetween.

### [BACKGROUND ART]

US 2007/114900 A1 discloses a spark plug having a multilayer firing tip including a discharge end and a weld end, with the weld end being connected to a center electrode, and more specifically to a base electrode on the center electrode. The weld end has a coefficient of thermal expansion, which is not between the values for the coefficients of thermal expansion for the discharge end and the base electrode. More specifically, the weld end has a coefficient of thermal expansion which is greater than the coefficients of thermal expansion for the discharge end and base electrode. The weld end is formed from Nickel and Chromium with a limited amount of additional elements. The spark plug is assembled by providing a first elongated material formed from the material used for the discharge end and a second elongated material formed from a material used for the weld end. The two materials are then joined to form a single joined material and are severed to create a firing tip. The firing tip is welded to the center electrode of the spark plug and more specifically, the base electrode.

As internal combustion engines such as automotive engines, for improving the fuel economy, high-efficiency engines are required which, for example, have low emissions and perform supercharging. In these high-efficiency engines, for improving the ignition performance, high-performance spark plugs are employed which have a discharge chip in at least one of a center electrode and a ground electrode.

As the discharge chip, for securing the wear resistance, noble metals such as Pt, Ir, Ru, Rh, Pd, Os or the like, or rare metals are used. However, in terms of cost reduction and suppression of the exhaustion of resources, it is requested, as an important issue, to reduce the use of high-melting point metals. As a measure on this issue, there have been proposed spark plugs in which the discharge chip is constituted of a clad material consisting of a base member-joining part joined to an electrode base member and a discharge part
facing a spark discharge gap. Moreover, in Patent Document 1, there is disclosed a method of manufacturing a discharge chip that is constituted of a clad material formed by joining a base member-joining part and a discharge part by both resistance welding and diffusion bonding.

### [PRIOR ART LITERATURE]

### [PATENT LITERATURE]

[PATENT DOCUMENT 1] WO2013015262A1

### [SUMMARY OF THE INVENTION]

### [PROBLEMS TO BE SOLVED BY THE INVENTION]

However, the discharge chip (clad electrode) disclosed in Patent Document 1 involves the following problems. Specifically, since the discharge chip is obtained by joining the discharge part and the base member-joining part, it is easy for a step to be formed therebetween. Accordingly, it is easy for a sharp corner portion of the base member-joining part to appear at a side portion of the discharge chip. Thus, when the discharge chip is used in a ground electrode or a center electrode of a spark plug, the strength of electric field will be high in the vicinity of the sharp corner portion of the base member-joining part. Consequently, it will be easy for discharge sparks to fly to the sharp corner portion of the base member-joining part at the side portion of the discharge chip; thus it may be difficult to form a normal discharge spark.

Therefore, it is desirable to eliminate the step between the discharge part and the base member-joining part. However, in the case of using the manufacturing method disclosed in Patent Document 1, it is difficult to obtain a discharge chip without a step. Specifically, in the manufacturing method, a noble metal chip (discharge part) is joined to a tape-shaped base material (base member-joining part) by resistance welding; then an integrated body of the base material and the noble metal chip is blanked out. Consequently, a step is formed between the noble metal chip and the base material. That is, after the blanking process, the diameter of the base material becomes greater than the diameter of the noble metal chip.

Moreover, if the discharge chip is made by blanking a composite plate that is obtained by bonding the material of the discharge part and the material of the base member-joining part, it is possible to result in the discharge chip having no step between the discharge part and the base member-joining part. However, in recycling the composite plate after the blanking process, it is necessary to separate the two different materials; thus there is a problem that the recycling cost becomes high.

In contrast, in the case of bonding the discharge part and the base member-joining part after blanking, to keep the joining area between the two parts constant, it is necessary to set the diameter of the base member-joining part to be greater than the diameter of the discharge part. Consequently, a step will be formed between the base member-joining part and the discharge part; thus a sharp corner portion of the base member-joining part will be formed at a side portion of the discharge chip.

The present invention has been made in view of the above circumstances, and aims to provide a method of manufacturing a spark plug for an internal combustion engine by which it is possible to suppress flying sparks to a base member-joining part.

### [MEANS FOR SOLVING THE PROBLEMS]

The present invention provides a method of manufacturing a spark plug for an internal combustion engine. In the spark plug, a center electrode and a ground electrode are opposed to each other with a spark discharge gap formed therebetween, and at least one of the center and ground electrodes has a discharge chip joined to an electrode base member so as to protrude toward the spark discharge gap. The method is characterized by comprising: a chip making step of making the discharge chip by joining a discharge part and a base member-joining part to each other, the discharge part being arranged on the spark discharge gap side, the base member-joining part being made of a material having a lower melting point than the discharge part and to be joined to the electrode base member; a temporary joining step of temporarily joining the discharge chip, at the base member-joining part, to the electrode base member by resistance welding; and a main joining step of joining, by laser welding, the discharge chip to the electrode base member so that a side surface of the discharge part and a surface of the electrode base member are smoothly connected by a connecting surface that has no sharp edge.

### [ADVANTAGEOUS EFFECTS OF THE INVENTION]

With the above method, in the obtained spark plug, no sharp corner portion of the base member-joining part appears at a side portion of the discharge chip. That is, it is possible to prevent a locally high-electric field strength portion from being formed in the base member-joining part. As a result, it is possible to suppress flying sparks to the base member-joining part.

Moreover, since the discharge chip is joined, by laser welding, to the electrode base member by melting and solidifying part of the base member-joining part and part of the electrode base member, it is particularly easy to have the outline of the base member-joining part shaped along the side surface of the discharge part and the surface of the electrode base member. Therefore, it is possible to easily join the discharge chip to the electrode base member so that the side surface of the discharge part and the surface of the electrode base member are smoothly connected.

As above, according to the present invention, it is possible to provide a method of manufacturing a spark plug for an internal combustion engine by which it is possible to suppress flying sparks to a base member-joining part.

### [BRIEF DESCRIPTION OF THE DRAWINGS]

FIG. 1 is a side view of a distal part of a spark plug in Example 1.
FIG. 2 (a) is a front view and FIG. 2(b) is a plan view of a discharge chip obtained by a chip making step in Example 1.
FIG. 3 is a front view showing a state where the discharge chip has been temporarily joined to an electrode base member by a temporary joining step in Example 1.
FIG. 4 is a front view showing a state where the discharge chip has been welded to the electrode base member by a main joining step in Example 1.
FIG. 5 is a schematic cross-sectional view illustrating how laser welding is performed in Example 1.
FIG. 6 is a schematic cross-sectional view showing the state where the discharge chip has been welded to the electrode base member by the main joining step in Example 1.
FIG. 7 is a side view of a distal part of a spark plug in Example 2.
FIG. 8 is a schematic cross-sectional view illustrating how laser welding is performed in Example 2.
FIG. 9 is a schematic cross-sectional view showing a state where a discharge chip has been welded to an electrode base member by a main joining step in Example 2.

### [EMBODIMENTS FOR CARRYING OUT THE INVENTION]

In the above-described spark plug for an internal combustion engine, the discharge chip may be included in the center electrode, in the ground electrode or in each of the center and ground electrodes.

The spark plug may be used, for example, as an ignition means in a combustion chamber of an internal combustion engine such as an automotive engine.

Moreover, in the discharge chip obtained in the chip making step, the diameter of the base member-joining part may be greater than the diameter of the discharge part. In this case, it is easy to stably perform the joining of the discharge part and the base member-joining part in the chip making step. However, in this case of the diameter of the base member-joining part being greater than the diameter of the discharge part, a step is formed between the two parts and a sharp corner portion of the base member-joining part appears. If the discharge chip was joined to the electrode base member so that the sharp corner portion remained appearing, it would be easy for discharge sparks of the spark plug to fly to the base member-joining part. Therefore, as described above, in the main joining step, by joining the discharge chip to the electrode base member so that the side surface of the discharge part and the surface of the electrode base member are smoothly connected by the connecting surface that has no sharp edge, the sharp corner portion of the base member-joining part can be eliminated. Consequently, it is possible to effectively suppress flying sparks to the base member-joining part.

### [Examples]

### (Example 1)

An example of the above method of manufacturing a spark plug for an internal combustion engine will be described with reference to FIGS. 1-6.

In a spark plug 1 obtained by the manufacturing method of the present example, as shown in FIG. 1, a center electrode 2 and a ground electrode 3 are opposed to each other with a spark discharge gap 11 formed therebetween. The center and ground electrodes 2 and 3 respectively have discharge chips 4 and 5 joined to electrode base members 20 and 30 so as to protrude toward the spark discharge gap 11.

In the present example, the discharge chip 5 in the ground electrode 3 is formed by joining a discharge part 51 arranged on the spark discharge gap 11 side and a base member-joining part 52 that is made of a material having a lower melting point than the discharge part 51 and joined to the electrode base member 30. On the other hand, the discharge chip 4 in the center electrode 2 is not a composite member.

The manufacturing method of the spark plug 1 of the present example includes a chip making step, a temporary joining step and a main joining step which will be described hereinafter. That is, via the following steps, the discharge chip 5 is joined to the electrode base member 30 to form the ground electrode 3.

In the chip making step, as shown in FIG. 2, the discharge chip 5 is made by joining the discharge part 51 and the base member-joining part 52 to each other. In the temporary joining step, as shown in FIG. 3, the discharge chip 5 is temporarily joined, at the base member-joining part 52, to the electrode base member 30 by resistance welding. In the main joining step, as shown in FIG. 4, the discharge chip 5 is joined, by laser welding, to the electrode base member 30 by melting and solidifying part of the base member-joining part 52 and part of the electrode base member 30, so that a side surface 511 of the discharge part 51 and a surface of the electrode base member 30 are smoothly connected by a connecting surface 523 that has no sharp edge.

As shown in FIG. 1, the electrode base member 30 of the ground electrode 3 extends distalward (i.e., downward in FIG. 1) from a distal end of a housing 12 of the spark plug 1 and is bent to a central axis side. The electrode base member 20 of the center electrode 2 is held inside an insulator 13 that is held inside the housing 12. Each of the housing 12 and the electrode base member 30 of the ground electrode 3 is made of a nickel alloy. Moreover, the electrode base member 20 of the center electrode 2 is also made of a nickel alloy.

Moreover, the electrode base member 30 of the ground electrode 3 has an opposing surface 31 that opposes the center electrode 2 in an axial direction of the spark plug 1 (to be simply referred to as "plug axial direction " hereinafter). To the opposing surface 31, there is joined the discharge chip 5. Moreover, to the distal end of the electrode base member 20 of the center electrode 2 which opposes the opposing surface 31 in the plug axial direction, there is joined the discharge chip 4. In the present example, the discharge chip 4 of the center electrode 2 is constituted, not of a composite member, but of, for example, a noble metal chip of an iridium alloy or the like. That is, the discharge chip 4 constituted of a noble metal chip is joined, for example by welding, to the distal end of the electrode base member 20 of the center electrode 2.

On the other hand, as described above, the discharge chip 5 of the ground electrode 3 is constituted of a composite member that is obtained by joining the discharge part 51 and the base member-joining part 52 to each other. In forming the ground electrode 3 that includes the discharge chip 5 constituted of the composite member, the above-described chip making step, the temporary joining step and the main joining step are performed. An example of each step will be described in detail hereinafter.

In the chip making step, first, the discharge part 51 made of a material having a relatively high melting point (e.g., the melting point being higher than or equal to 1700°C) and the base member-joining part 52 made of a material having a lower melting point than the discharge part 51 are prepared. As the material of the discharge part 51, it is possible to use, for example, Pt (Platinum), Ir (Iridium), Ru (Ruthenium), Rh (Rhodium), Pd (Palladium), Os (Osmium) or the like. Moreover, as the material of the base member-joining part 52, it is possible to use, for example, a Ni (Nickel) alloy. In addition, as the Ni alloy, it is possible to use one which has a melting point of, for example, 1400-1450°C.

Those metal members are processed, for example by blanking, to respectively form the cylindrical discharge part 51 and base member-joining part 52. Moreover, the diameter of the base member-joining part 52 is greater than the diameter of the discharge part 51.

The cylindrical discharge part 51 and base member-joining part 52 formed in the above manner are axially superposed with the central axes of the two parts coinciding with each other, as shown in FIG. 2. Then, in a state of the two parts being pressed against each other, a heat treatment is performed to join the discharge part 51 and the base member-joining part 52 by diffusion bonding. Consequently, the discharge chip 5 is obtained as a composite member. Therefore, in the vicinity of the interface between the discharge part 51 and the base member-joining part 52 in the discharge chip 5, there is formed a diffusion layer (not shown) in which atoms of the materials of the discharge part 51 and the base member-joining part 52 are diffused to each other.

In the discharge chip 5 obtained in the chip making step, the diameter of the base member-joining part 52 is greater than the diameter of the discharge part 51. Therefore, in this stage, there is formed a step between the base member-joining part 52 and the discharge part 51; at the step, there exists a sharp corner portion 521 of the base member-joining part 52.

In the temporary joining step, as shown in FIG. 3, the discharge chip 5 obtained in the chip making step is temporarily joined to the opposing surface 31 of the electrode base member 30. The temporary joining is performed by resistance welding. Specifically, the discharge chip 5 is made to abut, on its base member-joining part 52-side surface, a predetermined position on the opposing surface 31 of the electrode base member 30. Then, with the discharge chip 5 and the electrode base member 30 sandwiched between a pair of resistance welding electrodes, electric current is supplied to flow between the discharge chip 5 and the electrode base member 30. Consequently, by the Joule heat, the discharge chip 5 is welded and thus temporarily joined to the electrode base member 30.

Next, in the main joining step, as shown in FIG. 4, the discharge chip 5 is joined to the electrode base member 30 by laser welding. Specifically, as shown in FIG. 5, a laser beam L is irradiated to the discharge chip 5 temporarily joined to the electrode base member 30 from the vicinity of the joining portion. Here, the laser beam L is irradiated from a plurality of locations over the entire circumference of the joining portion with respect to the electrode base member 30. Moreover, the laser welding is performed at a temperature lower than the melting point of the discharge part 51. That is, in the main joining step, part of the base member-joining part 52 and part of the electrode base member 30 are melted without melting the discharge part 51. Consequently, as shown in FIG. 6, on an outer periphery of the base member-joining part 52, there is formed an annular melt zone 522 where the base member-joining part 52 and the electrode base member 30 are melted together and solidified.

Moreover, by the laser welding, as shown in FIGS. 4 and 6, the sharp corner portion 521 (see FIGS. 3 and 5) of the base member-joining part 52 is eliminated in shape, and there is formed the connecting surface 523 that smoothly connects the side surface 511 of the discharge part 51 and the surface (i.e., the opposing surface 31) of the electrode base member 30. The connecting surface 523 has, on a cross section taken along a plane passing through the central axis of the discharge chip 5, such a shape as to smoothly connect a curve and a straight line and have no sharp edge.

Next, advantageous effects of the present example will be described.

In the above main joining step, the discharge chip 5 is joined, by laser welding, to the electrode base member 30 by melting and solidifying part of the base member-joining part 52 and part of the electrode base member 30. Consequently, the discharge chip 5 is joined to the electrode base member 30 so that the side surface 511 of the discharge part 51 and the opposing surface 31 of the electrode base member 30 are connected by the connecting surface 523 that has no sharp edge. Therefore, in the obtained spark plug 1, no sharp corner portion 521 (see FIG. 3) of the base member-joining part 52 exists at a side portion of the discharge chip 5; thus it is possible to prevent a locally high-electric field strength portion from being formed in the base member-joining part 52. As a result, it is possible to suppress flying sparks to the base member-joining part 52.

Moreover, as described above, since the discharge chip 5 is joined, by laser welding, to the electrode base member 30 by melting and solidifying part of the base member-joining part 52 and part of the electrode base member 30, it is particularly easy to have the outline of the base member-joining part 52 shaped along the side surface 511 of the discharge part 51 and the opposing surface 31 of the electrode base member 30, as shown in FIG. 4. Therefore, it is possible to easily join the discharge chip 5 to the electrode base member 30 so that the side surface 511 of the discharge part 51 and the opposing surface 31 of the electrode base member 30 are connected by the connecting surface 523 that has no sharp edge.

Moreover, in the discharge chip 5 (see FIG. 2) obtained in the chip making step, the diameter of the base member-joining part 52 is greater than the diameter of the discharge part 51. Consequently, it is easy to stably perform the joining of the discharge part 51 and the base member-joining part 52. That is, it is possible to easily have the whole of an end surface of the discharge part 51 abutting the base member-joining part 52; thus it is easy to make the joining area of the discharge part 51 to the base member-joining part 52 constant, thereby obtaining stable joining strength therebetween. However, in this case of the diameter of the base member-joining part 52 being greater than the diameter of the discharge part 51, a step is formed between the two parts and the sharp corner portion 521 of the base member-joining part 52 appears. If the discharge chip 5 was joined to the electrode base member 30 so that the sharp corner portion 521 remained appearing, it would be easy for discharge sparks of the spark plug 1 to fly to the base member-joining part 52. Therefore, as described above, in the main joining step, as shown in FIG. 4, the sharp corner portion 521 of the base member-joining part 52 is eliminated by joining the discharge chip 5 to the electrode base member 30 so that the side surface 511 of the discharge part 51 and the opposing surface 31 of the electrode base member 30 are connected by the connecting surface 523 that has no sharp edge. Consequently, it becomes possible to smoothly connect, by the connecting surface 523 that has no sharp edge, the side surface of the discharge chip 5 from the side surface 511 of the discharge part 51 to a surface (i.e., the opposing surface 31) of the electrode base member 30. As a result, it becomes possible to effectively suppress flying sparks to the base member-joining part 52.

Moreover, in the main joining step, the laser welding is performed at a temperature lower than the melting point of the discharge part 51. Consequently, it is possible to sufficiently secure the volume and shape of the discharge part 51 that is made of a high-melting point material, thereby securing the wear resistance of the spark plug 1.

As above, according to the present example, it is possible to provide a method of manufacturing a spark plug for an internal combustion engine by which it is possible to suppress flying sparks to a base member-joining part.

### (Example 2)

In this example, as shown in FIGS. 7-9, the discharge chip 4 of the center electrode 2 is also constituted of a composite member; the composite member is obtained by joining a discharge part 41 arranged on the spark discharge gap 11 side and a base member-joining part 42 that is made of a material having a lower melting point than the discharge part 41 and joined to the electrode base member 20.

Moreover, in forming the center electrode 2, a chip making step, a temporary joining step and a main joining step are performed as described in Example 1.

In the chip making step, as in the chip making step of Example 1, the discharge chip 4 is obtained by diffusion-bonding the discharge part 41 and the base member-joining part 42. Next, in the temporary joining step, as shown in FIG. 8, the discharge chip 4 is temporarily joined, by resistance welding, to a distal end surface 21 of the electrode base member 20 of the center electrode 2. Specifically, a distal part of the electrode base member 20 of the center electrode 2 before joining the discharge chip 4 is substantially cone-shaped and has, at its distal end, a flat surface perpendicular to the axial direction. To this flat surface which constitutes the distal end surface 21, the discharge chip 4 is temporarily joined with the base member-joining part 42 abutting the distal end surface 21.

Next, in the main joining step, the discharge chip 4 is joined to the electrode base member 20 by laser welding. At this time, an annular melt zone 422 is formed between the base member-joining part 42 of the discharge chip 4 and the electrode base member 20. Moreover, as shown in FIG. 9, a sharp corner portion 421 (see FIG. 8) of the base member-joining part 42 is eliminated in shape, and there is formed a connecting surface 423 that smoothly connects a side surface 411 of the discharge part 41 and a surface (i.e., a side surface 22 of the substantially cone-shaped part) of the electrode base member 20. The connecting surface 423 has, on a cross section taken along a plane passing through the central axis of the discharge chip 5, such a shape as to smoothly connect a curve and a straight line and have no sharp edge.

The others are the same as in Example 1. In addition, unless particularly specified, of the reference signs used in the present example and the drawings relating to the present example, those which are the same as the reference signs used in Example 1 designate the same components as in Example 1.

In the present example, in the center electrode 2 as well, it is possible to suppress discharge sparks from flying to the electrode base member 20. As a result, it is possible to more reliably generate normal discharge sparks between the discharge part 41 of the center electrode 2 and the discharge part 51 of the ground electrode 3.

In addition, the present example has the same advantageous effects as Example 1.

In addition, besides the above-described examples, it is also possible to, for example, constitute the discharge chip of the ground electrode with a metal chip that is not a composite member or provide no discharge chip in the ground electrode while configuring the center electrode in the same manner as in Example 2.

### [DESCRIPTION OF REFERENCE SIGNS]

1: spark plug
11: spark discharge gap
2: center electrode
20: electrode base member (of the center electrode)
3: ground electrode
30: electrode base member (of the ground electrode)
4: discharge chip (of the center electrode)
41: discharge part (of the center electrode)
42: base member-joining part (of the center electrode)
5: discharge chip (of the ground electrode)
51: discharge part (of the ground electrode)
52: base member-joining part (of the ground electrode)

## Claims

1. A method of manufacturing a spark plug (1) for an internal combustion engine,
wherein in the spark plug (1), a center electrode (2) and a ground electrode (3) are opposed to each other with a spark discharge gap (11) formed therebetween, and at least one of the center and ground electrodes (2, 3) has a discharge chip (4, 5) joined to an electrode base member (20, 30) that is made of a Ni alloy, so as to protrude toward the spark discharge gap (11),
the method comprising:
a chip making step of making the discharge chip (4, 5) by joining a discharge part (41, 51) and a base member-joining part (42, 52) to each other, the discharge part (41, 51) being arranged on the spark discharge gap (11) side, the base member-joining part (42, 52) being made of a Ni alloy having a lower melting point than the discharge part (41, 51) and to be joined to the electrode base member (20, 30);
a temporary joining step of temporarily joining the discharge chip (4, 5), at the base member-joining part (42, 52), to the electrode base member (20, 30) by resistance welding, and
a main joining step of joining, by laser welding, the discharge chip (4, 5) to the electrode base member (20, 30) so that a side surface (411, 511) of the discharge part (41, 51) and a surface (22, 31) of the electrode base member (20, 30) are smoothly connected by a connecting surface (423, 523) that has no sharp edge,
wherein
in the main joining step, part of the base member joining part (42, 52) and part of the electrode base member (20, 30) are melted without melting the discharge part (41, 51),
in the discharge chip (4, 5) obtained in the chip making step, a diameter of the base member-joining part (42, 52) is greater than a diameter of the discharge part (41, 51), and
in the main joining step, the laser welding is performed at a temperature lower than the melting point of the discharge part (41, 51).

## Patentansprüche

1. Verfahren zum Herstellen einer Zündkerze (1) für eine Verbrennungskraftmaschine,
wobei in der Zündkerze (1), eine Mittelelektrode (2) und eine Masseelektrode (3) einander gegenüberliegen, wobei eine Zündfunkenstrecke (11) dazwischen ausgebildet ist, und zumindest eine von den Mittel- und Masseelektroden (2, 3) einen Entladungschip (4, 5) aufweist, der mit einem Elektrodensockelelement (20, 30) verbunden ist, das aus einer Ni-Legierung besteht, so dass es in Richtung der Zündfunkenstrecke (11) hervorsteht,
wobei das Verfahren aufweist:
einen Chipherstellungsschritt, in dem der Entladungschip (4, 5) hergestellt wird, indem ein Entladungsteil (41, 51) und ein Sockelelement-Verbindungsteil (42, 52) miteinander verbunden werden, wobei der Entladungsteil (41, 51) auf der Seite der Zündfunkenstrecke (11) angeordnet ist, der Sockelelement-Verbindungsteil (42, 52) aus einer Ni-Legierung besteht, die einen niedrigeren Schmelzpunkt aufweist als der Entladungsteil (41, 51), und mit dem Elektrodensockelelement (20, 30) verbunden wird;
einen temporären Verbindungsschritt, in dem der Entladungschip (4, 5) an dem Sockelelement-Verbindungsteil (42, 52) temporär mit dem Elektrodensockelelement (20, 30) durch Widerstandsschweißen verbunden wird, und
einen Hauptverbindungsschritt, in dem der Entladungschip (4, 5) mit dem Elektrodensockelelement (20, 30) durch Laserschweißen verbunden wird, so dass eine Seitenoberfläche (411, 511) des Entladungsteils (41, 51) und eine Oberfläche (22, 31) des Elektrodensockelelements (20, 30) reibungslos durch eine Verbindungsoberfläche (423, 523) verbunden werden, die keine scharfen Kanten aufweist,
wobei
in dem Hauptverbindungsschritt ein Teil des Sockelelement-Verbindungsteils (42, 52) und ein Teil des Elektrodensockelelements (20, 30) geschmolzen werden, ohne den Entladungsteil (41, 51) zu schmelzen,
bei dem Entladungschip (4, 5), der durch den Chipherstellungsschritt erhalten wird, ein Durchmesser des Sockelelement-Verbindungsteils (42, 52) größer ist als ein Durchmesser des Entladungsteils (41, 51), und
in dem Hauptverbindungsschritt das Laserschweißen bei einer Temperatur durchgeführt wird, die niedriger ist als der Schmelzpunkt des Entladungsteils (41, 51)

## Revendications

1. Procédé de fabrication d'une bougie d'allumage (1) pour un moteur à combustion interne,
dans lequel, dans la bougie d'allumage (1), une électrode centrale (2) et une électrode de masse (3) sont l'une en face de l'autre avec un espace de décharge à étincelle (11) formé entre elles, et au moins l'une des électrodes centrale et de masse (2, 3) comporte une pastille de décharge (4, 5) jointe à un élément de base d'électrode (20, 30) qui est constitué d'un alliage de Ni, de manière à faire saillie vers l'espace de décharge à étincelle (11),
le procédé comprenant :
une étape de fabrication de pastille pour fabriquer la pastille de décharge (4, 5) en joignant une partie de décharge (41, 51) et une partie de jonction d'élément de base (42, 52) l'une à l'autre, la partie de décharge (41, 51) étant agencée du côté de l'espace de décharge à étincelle (11), la partie de jonction d'élément de base (42, 52) étant constituée d'un alliage de Ni ayant un point de fusion inférieur à celui de la partie de décharge (41, 51) et destinée à être jointe à l'élément de base d'électrode (20, 30) ;
une étape de jonction temporaire pour joindre temporairement la pastille de décharge (4, 5), au niveau de la partie de jonction d'élément de base (42, 52), à l'élément de base d'électrode (20, 30) par soudage par résistance, et
une étape de jonction principale pour joindre, par soudage au laser, la pastille de décharge (4, 5) à l'élément de base d'électrode (20, 30) de sorte qu'une surface latérale (411, 511) de la partie de décharge (41, 51) et une surface (22, 31) de l'élément de base d'électrode (20, 30) soient reliées régulièrement par une surface de liaison (423, 523) qui n'a pas de bord tranchant,
dans lequel
à l'étape de jonction principale, une partie de la partie de jonction d'élément de base (42, 52) et une partie de l'élément de base d'électrode (20, 30) sont fondues sans fondre la partie de décharge (41, 51),
dans la pastille de décharge (4, 5) obtenue à l'étape de fabrication de pastille, un diamètre de la partie de jonction d'élément de base (42, 52) est plus grand qu'un diamètre de la partie de décharge (41, 51), et
à l'étape de jonction principale, le soudage au laser est effectué à une température inférieure au point de fusion de la partie de décharge (41, 51),
